



US005451561A

**United States Patent** [19]

Campbell et al.

[11] **Patent Number:** **5,451,561**[45] **Date of Patent:** **Sep. 19, 1995**[54] **RECEIVING ELEMENT SUBBING LAYER  
FOR THERMAL DYE TRANSFER**[75] Inventors: **Bruce C. Campbell; Teh-Ming Kung,  
both of Rochester; Kin K. Lum,  
Webster, all of N.Y.**[73] Assignee: **Eastman Kodak Company,  
Rochester, N.Y.**[21] Appl. No.: **294,293**[22] Filed: **Aug. 23, 1994**[51] Int. Cl.<sup>6</sup> ..... **B41M 5/035; B41M 5/38**[52] U.S. Cl. ..... **503/227; 428/195;  
428/211; 428/213; 428/318.4; 428/328;  
428/341; 428/342; 428/478.2; 428/913;  
428/914**[58] **Field of Search** ..... **8/471; 428/195, 328,  
428/330, 478.2, 913, 914, 211-213, 341, 342;  
503/227**

[56]

**References Cited****U.S. PATENT DOCUMENTS**4,992,414 2/1991 Kishida et al. ..... 503/227  
5,244,861 9/1993 Campbell et al. ..... 503/227*Primary Examiner*—Bruce H. Hess*Attorney, Agent, or Firm*—Harold E. Cole

[57]

**ABSTRACT**

Thermal dye transfer receiving elements are disclosed comprising a base having thereon a dye image-receiving layer, the base comprising a composite film laminated to a support, the dye image-receiving layer being on the composite film side of the base. The composite film comprises a microvoided thermoplastic core layer and at least one substantially void-free thermoplastic surface (skin) layer, and wherein there is a subbing layer between the thermoplastic surface layer and the dye image-receiving layer, the subbing layer comprising gelatin and titanium dioxide.

**20 Claims, No Drawings**

## RECEIVING ELEMENT SUBBING LAYER FOR THERMAL DYE TRANSFER

This invention relates to dye-receiving elements used in thermal dye transfer, and more particularly to a subbing layer for a microvoided composite film used as a support for a dye-receiving element which has a reduced pearlescence and gloss.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta and yellow signals. The process is then repeated for the other two colors. A color hard copy is thus obtained which corresponds to the original picture viewed on a screen. Further details of this process and an apparatus for carrying it out are contained in U.S. Pat. No. 4,621,271, the disclosure of which is hereby incorporated by reference.

Dye-receiving elements used in thermal dye transfer generally comprise a polymeric dye image-receiving layer coated on a base or support. In a thermal dye transfer printing process, it is desirable for the finished prints to compare favorably with color photographic prints in terms of image quality. The thermal dye receiver base must possess several characteristics for this to happen. First of all, transport through the printer is largely dependent on the base properties. The base must have low curl and a stiffness that is neither too high nor too low. The base has a major impact on image quality. Image uniformity is very dependent on the conformability of the receiver base. The efficiency of thermal transfer of dye from the donor to the receiver is also impacted by the base's ability to maintain a high temperature at its surface. The look of the final print is largely dependent on whiteness and surface texture of the base. Receiver curl before and after printing must be minimized. Cellulose paper, synthetic paper, and plastic films have all been proposed for use as dye-receiving element supports in efforts to meet these requirements.

In U.S. Pat. No. 5,244,861, dye-receiving elements are disclosed wherein a dye image-receiving layer is coated onto a composite film laminated to a support. The composite film comprises a microvoided thermoplastic core layer and at least one substantially void-free thermoplastic surface layer. However, there is a problem with these receivers because of undesirable pearlescence and gloss in the printed images. It is an object of this invention to reduce the pearlescence and gloss of such composite film receivers.

These and other objects are achieved in accordance with the invention, which comprises a dye-receiving element for thermal dye transfer comprising a base having thereon a dye image-receiving layer, the base

comprising a composite film laminated to a support, the dye image-receiving layer being on the composite film side of the base, the composite film comprising a microvoided thermoplastic core layer and a substantially void-free thermoplastic surface layer, the thermoplastic surface layer being adjacent to the dye image-receiving layer, and wherein there is a subbing layer between the thermoplastic surface layer and the dye image-receiving layer, the subbing layer comprising gelatin and titanium dioxide.

It has been found unexpectedly that a subbing layer comprising gelatin and titanium dioxide ( $TiO_2$ ) which is coated on one of the surface skin layers of a coextruded composite film used as support for a dye-receiving layer will substantially reduce the undesirable pearlescence and gloss phenomena which ordinarily would be observed in the printed images obtained with this type of unsubbed receiver supports.

The titanium dioxide which is in the subbing layer may be present in any amount which is effective for the intended purpose. In general, good results have been obtained when the titanium dioxide is present in an amount of from about  $0.10\text{ g}/\text{m}^2$  to about  $2.0\text{ g}/\text{m}^2$  of the subbing layer. Anatase or rutile titanium dioxide may be used such as Unitane ® 0-310 or Kemira 0220 ®  $TiO_2$ , anatase form, made by Kemira Corporation, Kronos 1072 ® (Kronos Inc.), Sachtleben LOCH-K ® (Sachtleben Chemie GmbH.) and Tioxide A-HR ® (Tioxide Inc.).

The gelatin in the subbing layer may be present in any amount which is effective for the intended purpose. In general, good results have been obtained when the gelatin is present in an amount of from about  $0.05$  to about  $1.1\text{ g}/\text{m}^2$  of the layer. Any type of gelatin can be used in the invention, such as bone gelatin or pigs skin gelatin.

Due to their relatively low cost and good appearance, these composite films are generally used and referred to in the trade as "packaging films." The support may include cellulose paper, a polymeric film or a synthetic paper. A variety of dye-receiving layers may be coated on these bases.

Unlike synthetic paper materials, microvoided packaging films can be laminated to one side of most supports and still show excellent curl performance. Curl performance can be controlled by the beam strength of the support. As the thickness of a support decreases, so does the beam strength. These films can be laminated on one side of supports of fairly low thickness/beam strength and still exhibit only minimal curl.

The low specific gravity of microvoided packaging films (preferably between  $0.3\text{--}0.7\text{ g}/\text{cm}^3$ ) produces dye-receivers that are very conformable and results in low mottle-index values of thermal prints as measured on an instrument such as the Tobias Mottle Tester. Mottle-index is used as a means to measure print uniformity, especially the type of nonuniformity called dropouts which manifests itself as numerous small unprinted areas. These microvoided packaging films also are very insulating and produce dye-receiver prints of high dye density at low energy levels. The non-voided skin produces receivers of high gloss and helps to promote good contact between the dye-receiving layer and the dye-donor film. This also enhances print uniformity and efficient dye transfer.

Microvoided composite packaging films are conveniently manufactured by coextrusion of the core and surface layers, followed by biaxial orientation, whereby voids are formed around void-initiating material con-

tained in the core layer. Such composite films are disclosed in, for example, U.S. Pat. No. 4,377,616, the disclosure of which is incorporated by reference.

The core of the composite film should be from 5 to 95% of the total thickness of the film, preferably from 30 to 85% of the total thickness. The non-voided skin(s) should thus be from 5 to 85% of the film, preferably from 15 to 70% of the thickness. The density (specific gravity) of the composite film should be between 0.2 and 1.0 g/cm<sup>3</sup>, preferably between 0.3 and 0.7 g/cm<sup>3</sup>. As the core thickness becomes less than 30% or as the specific gravity is increased above 0.7 g/cm<sup>3</sup>, the composite film starts to lose useful compressibility and thermal insulating properties. As the core thickness is increased above 85% or as the specific gravity becomes less than 0.3 g/cm<sup>3</sup>, the composite film becomes less manufacturable due to a drop in tensile strength and it becomes more susceptible to physical damage. The total thickness of the composite film can range from 20 to 150  $\mu\text{m}$ , preferably from 30 to 70  $\mu\text{m}$ . Below 30  $\mu\text{m}$ , the microvoided films may not be thick enough to minimize any inherent non-planarity in the support and would be more difficult to manufacture. At thicknesses higher than 70  $\mu\text{m}$ , little improvement in either print uniformity or thermal efficiency is seen, and so there is not much justification for the further increase in cost for extra materials.

"Void" is used herein to mean devoid of added solid and liquid matter, although it is likely the "voids" contain gas. The void-initiating particles which remain in the finished packaging film core should be from 0.1 to 10  $\mu\text{m}$  in diameter, preferably round in shape, to produce voids of the desired shape and size. The size of the void is also dependent on the degree of orientation in the machine and transverse directions. Ideally, the void would assume a shape which is defined by two opposed and edge-contacting concave disks. In other words, the voids tend to have a lens-like or biconvex shape. The voids are oriented so that the two major dimensions are aligned with the machine and transverse directions of the film. The Z-direction axis is a minor dimension and is roughly the size of the cross diameter of the voiding particle. The voids generally tend to be closed cells, and thus there is virtually no path open from one side of the voided-core to the other side through which gas or liquid can traverse.

The void-initiating material may be selected from a variety of materials, and should be present in an amount of about 5-50% by weight based on the weight of the core matrix polymer. Preferably, the void-initiating material comprises a polymeric material. When a polymeric material is used, it may be a polymer that can be melt-mixed with the polymer from which the core matrix is made and that can form dispersed spherical particles as the solution is cooled down. Examples of this would include nylon dispersed in polypropylene, poly(butylene terephthalate) in polypropylene, or polypropylene dispersed in poly(ethylene terephthalate). If the polymer is preshaped and blended into the matrix polymer, the important characteristics are size and shape of the particles. Spheres are preferred and they can be hollow or solid. These spheres may be made from cross-linked polymers which are members selected from the group consisting of an alkenylaromatic compound having the general formula  $\text{Ar}-\text{C}(\text{R})=\text{CH}_2$ , wherein Ar represents an aromatic hydrocarbon group, or an aromatic halohydrocarbon group of the benzene series and R is hydrogen or methyl group; acrylate-type mono-

mers include monomers of the formula  $\text{CH}_2=\text{C}(\text{R}')-\text{C}(\text{O})(\text{OR})$  wherein R is selected from the group consisting of hydrogen and an alkyl group containing from about 1 to 12 carbon atoms, and R' is selected from the group consisting of hydrogen and methyl; copolymers of vinyl chloride and vinylidene chloride, acrylonitrile and vinyl chloride, vinyl bromide, vinyl esters having formula  $\text{CH}_2=\text{CH}(\text{O})\text{COR}$ , wherein R is an alkyl group containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid, dialkyl terephthalic or ester-forming derivatives thereof with a glycol of the series  $\text{HO}(\text{CH}_2)_n\text{OH}$  wherein n is a whole number within the range of 2-10 and having reactive olefinic linkages within the polymer molecule; the above described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate, and mixtures thereof.

Examples of typical monomers for making the cross-linked polymer include styrene, butyl acrylate, acrylamide, acrylonitrile, methyl methacrylate, ethylene glycol dimethacrylate, vinylpyridine, vinyl acetate, methyl acrylate, vinylbenzyl chloride, vinylidene chloride, acrylic acid, divinylbenzene, acrylamidomethylpropanesulfonic acid, vinyltoluene, etc. Preferably, the cross-linked polymer is polystyrene or poly(methyl methacrylate). Most preferably, it is polystyrene and the crosslinking agent is divinylbenzene.

Processes well-known in the art yield non-uniformly sized particles, characterized by broad particle size distributions. The resulting beads can be classified by screening the produced beads spanning the range of the original size distribution. Other processes such as suspension polymerization, limited coalescence, directly yield very uniformly sized particles.

The void-initiating materials may be coated with a slip agent to facilitate voiding. Suitable slip agents or lubricants include colloidal silica, colloidal alumina, and metal oxides such as tin oxide and aluminum oxide. The preferred slip agents are colloidal silica and alumina, most preferably, silica. The crosslinked polymer having a coating of slip agent may be prepared by procedures well known in the art. For example, conventional suspension polymerization processes wherein the slip agent is added to the suspension are preferred.

The void-initiating particles can also be inorganic spheres, including solid or hollow glass spheres, metal or ceramic beads or inorganic particles such as clay, talc, barium sulfate, calcium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties.

Suitable classes of thermoplastic polymers for the core matrix-polymer of the composite film include polyolefins, polyesters, polyamides, polycarbonates, cellulosic esters, polystyrene, polyvinyl resins, polysul-

fonamides, polyethers, polyimides, poly(vinylidene fluoride), polyurethanes, poly(phenylene sulfides), polytetrafluoroethylene, polyacetals, polysulfonates, polyester ionomers, and polyolefin ionomers. Copolymers and/or mixtures of these polymers can be used.

Suitable polyolefins include polypropylene, polyethylene, polymethylpentene, and mixtures thereof. Polyolefin copolymers, including copolymers of ethylene and propylene are also useful.

Suitable polyesters include those produced from aromatic, aliphatic or cycloaliphatic dicarboxylic acids of 4-20 carbon atoms and aliphatic or alicyclic glycols having from 2-24 carbon atoms. Examples of suitable dicarboxylic acids include terephthalic, isophthalic, phthalic, naphthalenedicarboxylic acid, succinic, glutaric, adipic, azelaic, sebacic, fumaric, maleic, itaconic, 1,4-cyclohexanedicarboxylic, sodiosulfoisophthalic acids and mixtures thereof. Examples of suitable glycols include ethylene glycol, propylene glycol, butanediol, pentanediol, hexanediol, 1,4-cyclohexanediethanol, diethylene glycol, other polyethylene glycols and mixtures thereof. Such polyesters are well known in the art and may be produced by well known techniques, e.g., those described in U.S. Pat. Nos. 2,465,319 and 2,901,466. Preferred continuous matrix polyesters are those having repeat units from terephthalic acid or naphthalenedicarboxylic acid and at least one glycol selected from ethylene glycol, 1,4-butanediol and 1,4-cyclohexanediethanol. Poly(ethylene terephthalate), which may be modified by small amounts of other monomers, is especially preferred. Other suitable polyesters include liquid crystal copolymers formed by the inclusion of suitable amounts of a co-acid component such as stilbenedicarboxylic acid. Examples of such liquid crystal copolymers are those disclosed in U.S. Pat. Nos. 4,420,607, 4,459,402 and 4,468,510.

Useful polyamides include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite films include cellulose nitrate, cellulose triacetate, cellulose diacetate, cellulose acetate propionate, cellulose acetate butyrate, and mixtures or copolymers thereof. Useful polyvinyl resins include poly(vinyl chloride), poly(vinyl acetal), and mixtures thereof. Copolymers of vinyl resins can also be utilized.

The composite film can be made with skin(s) of the same polymeric material as the core matrix, or it can be made with skin(s) of polymeric composition different from that of the core matrix. For compatibility, an auxiliary layer can be used to promote adhesion of the skin layer to the core.

Addenda may be added to the core matrix to improve the whiteness of these films. This would include any process which is known in the art including adding a white pigment, such as titanium dioxide, barium sulfate, clay, or calcium carbonate. This would also include adding optical brighteners or fluorescing agents which absorb energy in the UV region and emit light largely in the blue region, or other additives which would improve the physical properties of the film or the manufacturability of the film.

Coextrusion, quenching, orienting, and heat setting of these composite films may be effected by any process which is known in the art for producing oriented film, such as by a flat film process or by a bubble or tubular process. The flat film process involves extruding the

blend through a slit die and rapidly quenching the extruded web upon a chilled casting drum so that the core matrix polymer component of the film and the skin components(s) are quenched below their glass transition

temperatures (Tg). The quenched film is then biaxially oriented by stretching in mutually perpendicular directions at a temperature above the glass transition temperature of the matrix polymers and the skin polymers. The film may be stretched in one direction and then in a second direction or may be simultaneously stretched in both directions. After the film has been stretched it is heat set by heating to a temperature sufficient to crystallize the polymers while restraining the film to some degree against retraction in both directions of stretching.

By having at least one non-voided skin on the microvoided core, the tensile strength of the film is increased and makes it more manufacturable. It allows the films to be made at wider widths and higher draw ratios than when films are made with all layers voided. Coextruding the layers further simplifies the manufacturing process.

The microvoided packaging films described in U.S. Pat. No. 5,244,861 are suitable for the practice of the invention when they are laminated by extrusion, pressure, or other means to a support such as polyester, paper, synthetic paper, or another microvoided film.

The support to which the microvoided composite films are laminated for the base of the dye-receiving element of the invention may be a polymeric, synthetic paper, or cellulose fiber paper support, or laminates thereof.

Preferred cellulose fiber paper supports include those disclosed in U.S. Pat. No. 5,250,496, the disclosure of which is incorporated by reference. When using a cellulose fiber paper support, it is preferable to extrusion laminate the microvoided composite films using a polyolefin resin. During the lamination process, it is desirable to maintain minimal tension of the microvoided packaging film in order to minimize curl in the resulting laminated receiver support. The backside of the paper support (i.e., the side opposite to the microvoided composite film and receiver layer) may also be extrusion coated with a polyolefin resin layer (e.g., from about 10 to 75 g/m<sup>2</sup>), and may also include a backing layer such as those disclosed in U.S. Pat. Nos. 5,011,814 and 5,096,875, the disclosures of which are incorporated by reference. For high humidity applications (>50% RH), it is desirable to provide a backside resin coverage of from about 30 to about 75 g/m<sup>2</sup>, more preferably from 35 to 50 g/m<sup>2</sup>, to keep curl to a minimum.

In one preferred embodiment, in order to produce receiver elements with a desirable photographic look and feel, it is preferable to use relatively thick paper supports (e.g., at least 120  $\mu$ m thick, preferably from 120 to 250  $\mu$ m thick) and relatively thin microvoided composite packaging films (e.g., less than 50  $\mu$ m thick, preferably from 20 to 50  $\mu$ m thick, more preferably from 30 to 50  $\mu$ m thick).

In another embodiment of the invention, in order to form a receiver element which resembles plain paper, e.g. for inclusion in a printed multiple page document, relatively thin paper or polymeric supports (e.g., less than 80  $\mu$ m, preferably from 25 to 80  $\mu$ m thick) may be used in combination with relatively thin microvoided composite packaging films (e.g., less than 50  $\mu$ m thick, preferably from 20 to 50  $\mu$ m thick, more preferably from 30 to 50  $\mu$ m thick).

The dye image-receiving layer of the receiving elements of the invention may comprise, for example, a polycarbonate, a polyurethane, a polyester, poly(vinyl chloride), poly(styrene-co-acrylonitrile), polycaprolactone or mixtures thereof. The dye image-receiving layer may be present in any amount which is effective for the intended purpose. In general, good results have been obtained at a concentration of from about 1 to about 10 g/m<sup>2</sup>. An overcoat layer may be further coated over the dye-receiving layer, such as described in U.S. Pat. No. 4,775,657, the disclosure of which is incorporated by reference.

Dye-donor elements that are used with the dye-receiving element of the invention conventionally comprise a support having thereon a dye containing layer. Any dye can be used in the dye-donor employed in the invention provided it is transferable to the dye-receiving layer by the action of heat. Especially good results have been obtained with sublimable dyes. Dye donors applicable for use in the present invention are described, e.g., in U.S. Pat. Nos. 4,916,112, 4,927,803 and 5,023,228, the disclosures of which are incorporated by reference.

As noted above, dye-donor elements are used to form a dye transfer image. Such a process comprises image-wise heating a dye-donor element and transferring a dye image to a dye-receiving element as described above to form the dye transfer image.

In a preferred embodiment of the invention, a dye-donor element is employed which comprises a poly(ethylene terephthalate) support coated with sequential repeating areas of cyan, magenta and yellow dye, and the dye transfer steps are sequentially performed for each color to obtain a three-color dye transfer image. Of course, when the process is only performed for a single color, then a monochrome dye transfer image is obtained.

Thermal printing heads which can be used to transfer dye from dye-donor elements to the receiving elements of the invention are available commercially. There can be employed, for example, a Fujitsu Thermal Head (FTP-040 MCS001), a TDK Thermal Head F415 HH-1089 or a Rohm Thermal Head KE 2008-F3. Alternatively, other known sources of energy for thermal dye transfer may be used, such as lasers as described in, for example, GB Appln. 2,083,726A.

A thermal dye transfer assemblage of the invention comprises (a) a dye-donor element, and (b) a dye-receiving element as described above, the dye-receiving element being in a superposed relationship with the dye-donor element so that the dye layer of the donor element is in contact with the dye image-receiving layer of the receiving element.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought into register with the dye-receiving element and the process repeated. The third color is obtained in the same manner.

The following example is provided to further illustrate the invention.

#### EXAMPLE

Test samples of receiver elements were prepared in the following manner. The receiver support was made

by laminating OPPalyte® 350 TW (Mobil Chemical Co.) packaging film to a paper support. OPPalyte® 350 TW is a composite film (38 µm thick) (d=0.62) consisting of a microvoided and oriented polypropylene core (approximately 73% of the total film thickness), with a titanium dioxide pigmented, non-microvoided, oriented polypropylene layer on each side; the void-initiating material is poly(butylene terephthalate).

The packaging film may be laminated in a variety of ways (by extrusion, pressure, or other means) to a paper support. In the present context, it was extrusion-laminated with pigmented polyolefin onto a paper stock support described below: the pigmented polyolefin was polyethylene (12 g/m<sup>2</sup>) containing anatase titanium dioxide (12.5% by weight) and a benzoxazole optical brightener (0.05% by weight); the paper stock support was 137 µm thick and made from a 1:1 blend of Pontiac Maple 51 (a bleached maple hardwood kraft of 0.5 mm length weighted average fiber length), available from Consolidated Pontiac, Inc., and Alpha Hardwood Sulphite (a bleached red-alder hardwood sulfite of 0.69 mm average fiber length), available from Weyerhaeuser Paper Co. The backside of the paper stock support was coated with high-density polyethylene (30 g/m<sup>2</sup>).

Thermal dye-transfer receiving elements were prepared from the above receiver support by coating the following layers in order on the top surface of the microvoided film:

Subbing layers were coated as shown in Table 1: the subbing layer solutions were prepared by mixing a TiO<sub>2</sub> dispersion (Unitane® 0-310 TiO<sub>2</sub>, anatase form, made by Kemira Corporation) and gelatin melt (Kodak gelatin 9293) along with 0.03% (wt-%) Olin 10G® surfactant (polyglycidol surfactant made by Olin Chemical Company). Three dry laydown ratios of TiO<sub>2</sub> and gelatin were employed: 1:1, 2:1 and 3:1. Also various laydowns were coated and are shown in the Table below.

Onto this support was coated a dye-receiving layer containing Makrolon® KL3-1013 polyether-modified bisphenol-A polycarbonate block copolymer (Bayer AG) (1.83 g/m<sup>2</sup>), GE Lexan® 141-112 bisphenol-A polycarbonate (General Electric Co.) (1.61 g/m<sup>2</sup>), Fluorad FC-431® perfluorinated alkylsulfonamidoalkyl ester surfactant (3M Co.) (0.011 g/m<sup>2</sup>), di-n-butyl phthalate (0.33 g/m<sup>2</sup>), and diphenyl phthalate (0.33 g/m<sup>2</sup>) coated from methylene chloride.

The dye-receiving layer was then overcoated with a solvent mixture of methylene chloride and trichloroethylene; a polycarbonate random terpolymer of bisphenol A (50 mole %), diethylene glycol (49 mole %), and polydimethylsiloxane (1 mole %), (2500 MW) block units (0.22 g/m<sup>2</sup>); Fluorad FC-431® surfactant (0.017 g/m<sup>2</sup>); and DC-510® surfactant (Dow-Corning Corp.) (0.0083 g/m<sup>2</sup>).

The dye-donor element which was used with the dye-receiving elements according to this invention was a support having thereon a dye-containing layer, as disclosed in copending U.S. Ser. No. 241,313, filed May 10, 1994, the disclosure of which is hereby incorporated by reference. This application discloses a detailed description of the dye-donor and the printing process followed to produce images on thermal dye-transfer receiver elements.

The gloss and pearlescence data shown in the Table were collected by using the following methods:

The 60 degree gloss measurements shown in the fifth column of the Table were made with a Gardner Micro-

Tri-Gloss meter according to the ASTM Standard Test Method for Specular Gloss (D-523-89).

The goniospectrophotometer color measurement system GCMS-3X (manufactured by Murakami Color Research Laboratory) was used to determine the "FLOP" values shown in the Table. "FLOP" is defined as an effect seen in samples with some sort of reflection-modifying structure that produces color changes when lighting or viewing conditions are changed. Many papers exhibit these geometric reflection properties known as "pearlenscence" or metallic sheen.

Specifically, pearlenscence can be caused by a variation in lightness (the  $L^*$  value is defined by the Commission Internationale de l'Eclairage in CIE Publication No. 15.2 (1986)) at different viewing angles. A goniospectrophotometer, as the one that was used in the present work, serves to measure lightness at many receiving angles from a fixed incident angle (light source). Data were collected for all samples shown in the Table with a 45 degree incident light beam (D65 Illumination), and lightness ( $L^*$ ) measurements were made at 35 degrees to the normal,  $L^*_{35}$ , zero degrees to the normal,  $L^*_0$ , and -65 degrees to the normal,  $L^*_{-65}$ .

The following equation was used to calculate the FLOP values shown in the Table:

$$\frac{15 (L^*_{35} - L^*_{-65})^{1.11}}{L^*_0^{0.86}}$$

Higher FLOP values indicate a higher degree of pearlenscence. The following references provide more details:

- 1) D. H. Altman, "Directional Color measurement of Metallic Flake Finishes," paper delivered at the 1087 INTER-SOCIETY COLOR COUNCIL Conference on "Appearance," Feb. 8-11, 1987;
- 2) F. W. Billmeyer, Jr., and Francis X. D. O'Donnell, "Visual Gloss Scaling and Multidimensional Scaling Analysis of Painted Specimens," Color Research and Application, Vol. 12, No. 6, pp. 315-326 (Dec. 1987).

The following results were obtained:

TABLE\*

| SAMPLE ID | TiO <sub>2</sub> /GEL RATIO | TiO <sub>2</sub> COVERAGE g/m <sup>2</sup> | GEL COVERAGE g/m <sup>2</sup> | 60 DEGREE GLOSS | FLOP |
|-----------|-----------------------------|--------------------------------------------|-------------------------------|-----------------|------|
| C-1       | Control                     | 0                                          | 0.22                          | 113.3           | 12.5 |
| A         | 1:1                         | 0.13                                       | 0.13                          | 106.6           | 5.7  |
| B         | 1:1                         | 0.27                                       | 0.27                          | 103.5           | 1.9  |
| C         | 1:1                         | 0.60                                       | 0.60                          | 101.7           | 0.2  |
| D         | 1:1                         | 1.08                                       | 1.08                          | 101.5           | 0.0  |
| E         | 2:1                         | 0.09                                       | 0.04                          | 112.8           | 12.5 |
| F         | 2:1                         | 0.17                                       | 0.09                          | 105.4           | 4.7  |
| G         | 2:1                         | 0.37                                       | 0.18                          | 103.5           | 2.5  |
| H         | 2:1                         | 0.54                                       | 0.27                          | 101.9           | 0.5  |
| I         | 2:1                         | 0.81                                       | 0.41                          | 102.2           | 0.0  |
| J         | 2:1                         | 1.62                                       | 0.81                          | 100.8           | 0.0  |
| K         | 3:1                         | 0.19                                       | 0.07                          | 103.9           | 3.9  |
| L         | 3:1                         | 0.41                                       | 0.14                          | 102.5           | 1.5  |
| M         | 3:1                         | 0.90                                       | 0.30                          | 100.4           | 0.0  |
| N         | 3:1                         | 1.62                                       | 0.54                          | 73.2            | 0.0  |

\*Composition of the subbing layers varies as shown in columns 2-4.

The above data clearly show the beneficial effects of a TiO<sub>2</sub>-containing subbing layer between the microvoided support and image receiving layer. Also evident is the elimination of pearlenscence for higher TiO<sub>2</sub> laydowns, regardless of the TiO<sub>2</sub>/gel ratio (see the data for samples D, I, J, M, and N).

The invention has been described in detail with particular reference to preferred embodiments thereof, but

it will be understood that variations and modifications can be effected within the spirit and scope of the invention.

What is claimed is:

- 5 1. A dye-receiving element for thermal dye transfer comprising a base having thereon a dye image-receiving layer, the base comprising a composite film laminated to a support, the dye image-receiving layer being on the composite film side of the base, the composite film comprising a microvoided thermoplastic core layer and a substantially void-free thermoplastic surface layer, the thermoplastic surface layer being adjacent to the dye image-receiving layer, and wherein there is a subbing layer between said thermoplastic surface layer and said dye image-receiving layer, said subbing layer comprising gelatin and titanium dioxide.
- 15 2. The element of claim 1 wherein the thickness of the composite film is from 30 to 70  $\mu\text{m}$ .
- 20 3. The element of claim 1 wherein the core layer of the composite film comprises from 30 to 85% of the thickness of the composite film.
- 25 4. The element of claim 1 wherein the titanium dioxide is present in an amount of from about 0.10 to about 2.0 g/m<sup>2</sup> of the subbing layer.
- 30 5. The element of claim 1 wherein the gelatin is present in an amount of from about 0.05 to about 1.1 g/m<sup>2</sup> of the subbing layer.
- 35 6. The element of claim 1 wherein the composite film comprises a microvoided thermoplastic core layer having a substantially void-free thermoplastic surface layer on each side thereof.
- 40 7. The element of claim 1 wherein the support comprises synthetic paper.
8. The element of claim 1 wherein the support comprises a non-voided polymer film.
9. The element of claim 1 wherein the support comprises cellulose fiber paper.
- 45 10. The element of claim 9 wherein the paper support is from 120 to 250  $\mu\text{m}$  thick and the composite film is from 30 to 50  $\mu\text{m}$  thick.
11. The element of claim 9 further comprising a polyolefin backing layer on the side of the support opposite to the composite film.

12. The element of claim 11 wherein the polyolefin backing layer is present at a coverage of from 30 to 75 g/m<sup>2</sup>.

13. The element of claim 1 wherein the composite film comprises a microvoided and oriented polypropyl-

ene core layer with a surface layer of non-microvoided oriented polypropylene on each side.

14. The element of claim 13 wherein the support is a cellulose fiber paper support from 120 to 250  $\mu\text{m}$  thick and the composite film is from 30 to 50  $\mu\text{m}$  thick.

15. The element of claim 1 wherein the core layer of the composite film comprises a microvoided and oriented thermoplastic polymer and a polymeric void-initiating material.

16. A process of forming a dye transfer image comprising:

a) imagewise-heating a dye-donor element comprising a support having thereon a dye layer comprising a dye dispersed in a binder, and

b) transferring a dye image to a dye-receiving element comprising a base having thereon a dye image-receiving layer to form said dye transfer image,

wherein the dye-receiving element base comprises a composite film laminated to a support, the dye image-receiving layer being on the composite film side of the base, the composite film comprising a microvoided thermoplastic core layer and at least one substantially void-free thermoplastic surface layer, the thermoplastic surface layer being adjacent to the dye image-receiving layer, and wherein there is a subbing layer between said thermoplastic surface layer and said dye image-receiving layer, said subbing layer comprising gelatin and titanium dioxide.

17. The process of claim 16 wherein the composite film comprises a microvoided thermoplastic core layer having a substantially void-free thermoplastic surface

layer on each side thereof, the thickness of the composite film being from 30 to 70  $\mu\text{m}$ .

18. The process of claim 16 wherein the support comprises cellulose fiber paper from 120 to 250  $\mu\text{m}$  thick and the composite film is from 30 to 50  $\mu\text{m}$  thick and comprises a microvoided and oriented polypropylene core layer with a surface layer of non-microvoided oriented polypropylene on each side.

19. A thermal dye transfer assemblage comprising:

a) a dye-donor element comprising a support having thereon a dye layer comprising a dye dispersed in a binder, and

b) a dye-receiving element comprising a support having thereon a dye image-receiving layer, said dye-receiving element being in a superposed relationship with said dye-donor element so that said dye layer is in contact with said dye image-receiving layer,

wherein the dye-receiving element base comprises a composite film laminated to a support, the dye image-receiving layer being on the composite film side of the base, the composite film comprising a microvoided thermoplastic core layer and at least one substantially void-free thermoplastic surface layer, the thermoplastic

surface layer being adjacent to the dye image-receiving layer, and wherein there is a subbing layer between said thermoplastic surface layer and said dye image-receiving layer, said subbing layer comprising gelatin and titanium dioxide.

20. The assemblage of claim 19 wherein the thickness of the composite film is from 30 to 70  $\mu\text{m}$ .

\* \* \* \* \*